

## UNITED STATES PATENT OFFICE

2,335,758

PROCESS FOR REMOVAL OF ARSENIC  
FROM LEAD CONTAINING IT

Max F. W. Heberlein, Rahway, and Nevin R. Bierly, Avenel, N. J., assignors to The American Metal Company, Limited, New York, N. Y., a corporation of New York

No Drawing. Application March 5, 1942,  
Serial No. 433,464

5 Claims. (Cl. 75—78)

This invention relates to the removal of arsenic from impure lead, containing antimony and arsenic.

An important object of the invention is to provide a simple, efficient process for removing arsenic from lead containing antimony without removing appreciable quantities of lead or antimony with the arsenic and to provide an arsenic-containing slag having a low content of other metals.

Other objects will be in part obvious and in part pointed out hereinafter.

In accordance with our invention it is possible to remove arsenic with no substantial amount of antimony and only a small amount of lead. This is a distinct advantage over the older processes where antimony and arsenic are removed together and must be separated subsequently by tedious and expensive methods.

Although our process may be operated in the presence of tin, it is preferred not to have tin present. If present, it appears in the dross with the arsenic and must be separated by subsequent treatment.

In working our process accordingly, we prefer to use lead from which the tin has already been removed. Any process capable of a selective tin removal may, of course, be used. We prefer the Harper and Reinberg process as described in Patent No. 2,155,545 which is highly efficient for tin removal, bringing the tin content of the lead down to several hundredths of one per cent or traces of tin.

We have found in accordance with our invention that arsenic in lead containing arsenic and antimony can be converted into an oxidized compound, probably sodium arsenite, by sodium hydroxide, NaOH, without the aid of any other agent, while antimony will only react with sodium hydroxide after it has been oxidized by some oxidizing agent such as air, nitre, etc. Accordingly, a clean-cut separation of arsenic can be accomplished if a combination of arsenic, lead and antimony is treated with sodium hydroxide in the absence of air, whereby the arsenic is converted into a compound, probably arsenite, and can be removed by skimming.

A practical method of excluding air is to equip the well-known refining kettle, such as shown in the said Harper and Reinberg patent, with a tight-fitting cover. Experiments conducted with this type of equipment have shown that arsenic can be completely removed in the manner indicated from lead on a commercial scale without appreciably affecting the antimony or lead.

Arsenic contents of less than 0.01% in the treated metal have been obtained easily and the corresponding antimony contents equalled or approximated the antimony analyses of the original metals. The arsenic drosses removed in our process usually contain between 20 and 30% arsenic, and less than 1% each of antimony and lead.

In carrying out the process of our invention, 10 after the tin has been removed from the lead, it is preferably transferred to a kettle which is equipped with a simple air-tight cover. A layer of solid sodium hydroxide is placed on the molten lead bath. The stirrer is put into position in 15 the kettle, after which the air-tight cover is fastened to the kettle and the stirrer shaft. The cover may consist of a simple steel plate bolted or clamped to the kettle with an asbestos gasket between the cover and rim of the kettle. The stirrer shaft passes through a close-fitting opening in the center of the cover. Various modifications in the type of apparatus to insure the exclusion of air may of course be used. After the cover is firmly secured, the stirrer is started and the 20 caustic soda thoroughly stirred into the metal bath to insure intimate contact between the caustic and all parts of the metal bath. We believe the arsenic combines with the caustic to 25 form a dross of  $Na_3AsO_3$ , according to the equation



The dross is removed by skimming and will contain little lead and substantially no antimony. 35 During the treatment, hydrogen is liberated as above indicated and burned at a vent, such as a bleeder valve, provided in the kettle. As the hydrogen flame diminishes, it indicates that the elimination of arsenic approaches its completion.

40 Some of the arsenic dross when leached and the liquors analyzed for trivalent and pentavalent arsenic have shown that the arsenic occurs in this solution in varying percentages (30-60%) 45 in the trivalent form, but it is believed that during the kettle treatment under exclusion of air only  $Na_3AsO_3$  is formed but immediately upon removing the cover from the treatment kettle, this compound starts to oxidize and continues 50 during the skimming period to form  $Na_3AsO_4$ . Oxidation at this time is very likely because the dross is handled and exposed to the air, while it has a temperature of above 650-700° F. This elevated temperature accelerates any oxidation 55 and naturally would also promote the conversion

of trivalent arsenic into the pentavalent form.

We have found in accordance with our invention that the temperature to which the metal is heated has a direct bearing on the time required to remove the arsenic, all other conditions being the same. Thus, although we have operated our process below 900° F., we prefer to operate between 1000 and 1100° F., because the speed of removal is so much higher. As stated above, a layer of sodium hydroxide is placed on the molten metal at the proper temperature using approximately 2½ pounds for each pound of arsenic in the metal, which represents an excess of about 50% on the basis of  $\text{Na}_3\text{AsO}_3$  formation.

An ordinary stirrer operating around 300 R. P. M. may be used to agitate the bath or a high-speed impeller operating from 900 to 1700 R. P. M. as used in the Harper and Reinberg Patent No. 2,155,545 may be used. We prefer the high speed stirrer because it creates a more efficient and thorough mixing of the reacting substances. Other means of agitation may be employed if desired.

The time required for stirring depends on the temperature, type of stirring apparatus, amount of arsenic present and other indicated variables, but in our preferred practice with the usual grades of lead containing around ½% of arsenic, 1 to 2 hours stirring is usually sufficient to bring the arsenic content down to several hundredths of 1%. It may sometimes be desirable to remove only part of the arsenic, and in that event less reagent may be used and the stirring time correspondingly reduced. In order to determine whether the desired amount of arsenic has been removed, the metal is sampled and assayed. After operating the process for a short time, experience will soon teach the amount of reagent and the time required with a given set of conditions, in order to obtain the removal of arsenic desired.

After stirring for the desired length of time, the slag is skimmed off and leached with hot water after which it is filtered. The relatively small amount of residue or filter cake which contains some lead and antimony may be returned to the lead smelter for the recovery of values contained. The filtrate containing the arsenic substantially free from other metals may be discarded, or may be converted to some form suitable for sale. Arsenic slags produced by previous processes have been contaminated by other metals requiring further treatment to obtain the other metals or the arsenic or both.

The method which we have preferably used in order to exclude the air from the reaction has been the application of a simple tight-fitting cover as described above. However, in addition to a cover, an atmosphere of a neutral gas in the chamber between the top of the lead bath and the tight-fitting cover may be provided, if desired. In this case an inlet, as well as an outlet pipe must be connected to the cover, so that the neutral gas can be fed in at the inlet and, by having the outlet just slightly open, the gas can be kept under a slight pressure at all times. The introduction of a neutral gas, particularly at the end of the operation, will avoid sucking in of air under the cover and will eliminate possible explosion of hydrogen.

In the commencement of the process, or at any time if desired, fresh sodium hydroxide may be employed for the elimination of the arsenic. It is preferable, however, to operate so that the

fresh caustic is placed on the bath of metal after a considerable proportion of the arsenic has been removed from the metal bath by the process. In other words, after the arsenic content

5 has been built up to a high point in the dross, this dross is skimmed off from the metal bath and then fresh caustic soda containing preferably no arsenic is shoveled onto the bath and the final proportion of arsenic in the molten metal is removed. The dross then formed will consist of caustic soda with a small amount of arsenic content. Then on the next batch of 10 fresh metal treated, this caustic soda containing a small arsenic content, which content may be still further reduced by addition of fresh sodium hydroxide thereto if desired, is first placed on the bath and the process conducted so that a large proportion of the arsenic content is removed. At this point, then, following the procedure mentioned above, fresh sodium hydroxide is shoveled on and the process so continued.

15 Arsenic in the bullion can be readily reduced to traces by this method and final slags with very little antimony and lead can be made.

The following are examples of the process as we now prefer to practise it. The invention is not to be considered as limited thereby except as indicated in the appended claims.

#### EXAMPLE 1

20 7,740 lbs. of metal assaying .36% As, 6.16% Sb and the balance substantially lead, were placed in a kettle and melted down and the temperature raised to about 1000° F. To this was added 80 lbs. of fresh sodium hydroxide which is equivalent to about 2.8 lbs. of hydroxide per pound of arsenic. The impeller was placed in the molten metal bath and the steel-plate cover device placed on the kettle to exclude the air. The stirrer provided with a 6½ inch impeller was run at a speed of 1700 R. P. M. for 2 hours with the metal bath between 1000 and 1100° F. A sample of the metal taken after 1 hour of stirring showed the arsenic to be reduced to .07%, while at the end of the second hour the arsenic was reduced to .03%.

25 At the end of two hours the liquid dross was removed, weighed and analyzed.

30 The following metal balance shows the results obtained:

| 55 | Material              | Amount | Analysis, per cent |      |      |
|----|-----------------------|--------|--------------------|------|------|
|    |                       |        | As                 | Sb   | Pb   |
|    |                       |        | Bal.               | Bal. | Bal. |
|    | Head metal            | 7,740  | .36                | 6.16 |      |
|    | Sodium hydroxide slag | 114    | 22.10              | .49  | .51  |
|    | Final metal           | 7,700  | .03                | 5.81 | Bal. |

35 60 The rate of removal of the first hour and second hour based on metal assays is as follows:

| 65 | Metal        | Weight | Per cent As | Pounds As | Pounds arsenic removed |            | Rate of removal of arsenic, pounds per hour per ton |            |
|----|--------------|--------|-------------|-----------|------------------------|------------|-----------------------------------------------------|------------|
|    |              |        |             |           | Per hour               | Cumulative | Per hour                                            | Cumulative |
|    |              |        |             |           |                        |            |                                                     |            |
| 70 | At start     | 7,740  | .36         | 27.86     |                        |            |                                                     |            |
|    | After 1 hr.  | 7,720  | .07         | 5.40      | 22.46                  |            | 5.83                                                |            |
|    | After 2 hrs. | 7,700  | .03         | 2.31      | 3.09                   | 25.55      | .8                                                  | 3.30       |

75 The assays of the caustic dross removed show the very excellent removal of arsenic with a very small removal of antimony and lead. The actual

ratio of arsenic to antimony in the dross made on this run was 45 to 1 and of arsenic to lead 43 to 1.

The results also show that over 90% of the arsenic was removed in a short time by our simple process.

#### EXAMPLE 2

The following is a two-step process for reducing arsenic to a trace:

Step 1.—To 7,380 lbs. of lead containing .88% arsenic, .73% antimony, balance substantially lead and contained in a kettle as in Example 1 with air excluded, was added 185 lbs. fresh sodium hydroxide during the first fifteen minutes of stirring. Stirring was carried on at the rate of 1700 R. P. M. with a 6½ inch impeller. The temperature at the start of the stirring period was 850° F. and this was gradually raised to 1100° F. After 5 hours of stirring, the metal assayed .13% As and after 6 hours, it assayed .10% As. The slag was removed at the end of 6 hours. It was liquid, weighed 222 lbs. and assayed 29.13% As, .46% Sb and a trace of lead.

Step 2.—To the metal remaining in the kettle after 6 hours stirring was added 100 lbs. of fresh sodium hydroxide and after stirring 50 minutes, the metal contained only a trace of arsenic. The slag removed at that time weighed 115 lbs. and assayed 9.58% arsenic, .91% antimony and .20% lead. This slag may be charged to a new batch of lead, containing arsenic, to be treated or otherwise disposed of.

The following is a tabulation of the results obtained from these steps:

#### Step 1

| Material                           | Amount       | Time    | Analysis, per cent |     |       |
|------------------------------------|--------------|---------|--------------------|-----|-------|
|                                    |              |         | As                 | Sb  | Pb    |
| Head metal.....                    | Pounds 7,380 | Hours 0 | .88                | .73 | Bal.  |
| Final metal.....                   | 7,320        | 6       | .10                | .60 | Bal.  |
| Sodium hydroxide caustic slag..... | 222          | 6       | 29.13              | .46 | Trace |

#### Step 2

| Material          | Amount       | Time    | Analysis, per cent |     |      |
|-------------------|--------------|---------|--------------------|-----|------|
|                   |              |         | As                 | Sb  | Pb   |
| Head metal.....   | Pounds 7,320 | Hours 0 | .10                | .60 | Bal. |
| Final metal.....  | 7,295        | 56      | Trace              | .57 | Bal. |
| Counter slag..... | 115          | 56      | 9.58               | .91 | .20  |

#### EXAMPLE 3

The following example shows the use of (a) fresh sodium hydroxide on a lead-arsenic bath to produce a dross having a low arsenic content, and (b) the use of this dross on a second bath to produce a second dross having a higher arsenic content. This second metal bath is then treated with fresh hydroxide to produce a dross having a low metal content and then the process is repeated using this low arsenic dross on a new metal bath as in step b. To 54,888 parts of metal assaying .241% of arsenic and .65% of antimony and the remainder lead, there was added 975 parts of fresh sodium hydroxide to produce a dross containing 8.43% arsenic and 2.42% antimony. The final metal carried less than .005% arsenic and .60% antimony. These figures are set forth in Table a below and it will be noted

that the original metal is designated as "(a) Head metal"; the sodium hydroxide is designated as "(a) NaOH (hydroxide)"; the dross as "(a) Dross," and the final metal as "(a) Final metal."

Table a

| Parts                     | Analysis, per cent |                |         |
|---------------------------|--------------------|----------------|---------|
|                           | As                 | Sb             | Pb      |
| (a) Head metal.....       | 54,888             | .241           | .65     |
| (a) NaOH (hydroxide)..... | 975                | -----          | -----   |
| (a) Dross.....            | 1,385              | 8.43           | 2.42    |
| (a) Final metal.....      | 54,445             | Less than .005 | .60     |
|                           |                    | -----          | Balance |

In carrying out step b above, (a) dross was then put on a fresh metal bath and the process continued, to produce a dross which was then removed; whereupon fresh sodium hydroxide was added to produce a dross and final metal, and this dross was then available for use with a head metal such as that employed at the start of step b.

The 1,385 parts of (a) dross above was accordingly added to 54,940 parts of lead containing .577% arsenic and .6% antimony and after stirring with air excluded, there were produced 1,365 parts of dross assaying 23.2% arsenic, .75% antimony, .64% lead. The 54,940 parts of lead mentioned in step b are designated as "(b) Head metal" in Table b below. The dross produced by this step b is designated as "(b) Dross" in said table. After removal of the (b) dross, a second treatment of the remaining metal with 425 parts of fresh sodium hydroxide reduced the arsenic content of the said metal to less than .005%. In Table b this sodium hydroxide is designated as "Fresh NaOH"; the dross is designated as "(c) Dross" and the metal obtained is designated as "(b) Final metal." (b) Dross may then be treated to recover the arsenic or thrown away and (c) Dross may be put on a fresh bath of metal containing relatively large quantities of arsenic to be removed, such as (a) or (b) Head metal above, and the process then continued to remove this arsenic. When the arsenic content of this dross has risen sufficiently, it is then removed and fresh sodium hydroxide placed on the metal to reduce the arsenic content to somewhere in the neighborhood of .005%. In other words, the process is a cyclic one, as indicated in the statement at the beginning of this example.

Results of this run are shown in the following table:

Table b

| Parts                       | Analysis, per cent |                |         |
|-----------------------------|--------------------|----------------|---------|
|                             | As                 | Sb             | Pb      |
| (b) Head metal.....         | 54,940             | .577           | .60     |
| (a) Dross.....              | 1,385              | 8.43           | 2.42    |
| (b) Dross.....              | 1,365              | 23.2           | .75     |
| Fresh NaOH (hydroxide)..... | 425                | -----          | .64     |
| (c) Dross.....              | 795                | 16.3           | 1.3     |
| (b) Final metal.....        | 54,810             | Less than .005 | .60     |
|                             |                    | -----          | Balance |

Instead of sodium hydroxide mentioned in the above examples, we may also employ other caustic alkali such as potassium hydroxide, but we prefer sodium hydroxide because of its lower cost.

What we claim is:

1. A process for treating impure lead containing arsenic and antimony which comprises melting the impure lead, agitating it with caustic alkali substantially in the absence of air in con-

tact with any part of the bath and forming a dross containing arsenic but with no substantial amount of antimony.

2. A process for treating impure lead containing arsenic and antimony which comprises stirring the impure lead in molten condition with caustic alkali substantially in the absence of air in contact with any part of the bath while maintaining a temperature of the order of 1000-1100° F. and forming a dross containing arsenic but with no substantial amount of antimony. 10

3. A process for treating impure lead containing arsenic and antimony which comprises agitating the impure molten lead with sodium hydroxide while maintaining the temperature at about 1000-1100° F. substantially in the absence of air in contact with any part of the bath and forming a dross containing arsenic but with no substantial amount of antimony. 15

4. A process for treating impure lead containing arsenic and antimony which comprises melting the impure lead in an air-tight kettle and stirring it substantially in the absence of air in contact with any part of the bath with caustic alkali and forming a dross containing arsenic but with only a small amount of antimony.

5. A process for treating impure lead containing arsenic and antimony which comprises melting the impure lead in an air-tight kettle and stirring it substantially in the absence of air in contact with any part of the bath while maintaining a temperature at about 1000-1100° F. with sodium hydroxide, and forming a dross containing arsenic but with only a small amount of antimony.

MAX F. W. HEBERLEIN.  
NEVIN R. BIERLY.